



US007862978B2

(12) **United States Patent**  
**Morris et al.**

(10) **Patent No.:** **US 7,862,978 B2**  
(b4) **Date of Patent:** **\*Jan. 4, 2011**

(54) **TONER AND MANUFACTURING PROCESS THEREFOR**

(75) Inventors: **Daniel Patrick Morris**, Manchester (GB); **Martin Russell Edwards**, Manchester (GB); **Mohammed Nawaz**, Manchester (GB); **Oliver Callaghan**, Manchester (GB); **Simon Pickard**, Cheadle (GB)

(73) Assignee: **Fujifilm Imaging Colorants Limited**, Manchester (GB)

(\*) Notice: Subject to any disclaimer, the term of this patent is extended or adjusted under 35 U.S.C. 154(b) by 57 days.

This patent is subject to a terminal disclaimer.

(21) Appl. No.: **12/083,502**

(22) PCT Filed: **Nov. 6, 2006**

(86) PCT No.: **PCT/GB2006/004142**

§ 371 (c)(1),  
(2), (4) Date: **Apr. 11, 2008**

(87) PCT Pub. No.: **WO2007/052062**

PCT Pub. Date: **May 10, 2007**

(65) **Prior Publication Data**

US 2009/0162774 A1 Jun. 25, 2009

(30) **Foreign Application Priority Data**

Nov. 7, 2005 (GB) ..... 0522650.1

(51) **Int. Cl.**

**G03G 9/00** (2006.01)

(52) **U.S. Cl.** ..... **430/137.14; 430/108.1;**  
**430/110.1; 430/137.1**

(58) **Field of Classification Search** ..... **430/108.1,**  
**430/110.1, 137.1, 137.14**

See application file for complete search history.

(56) **References Cited**

U.S. PATENT DOCUMENTS

- |                   |         |                              |
|-------------------|---------|------------------------------|
| 4,983,488 A       | 1/1991  | Tan et al.                   |
| 4,996,127 A       | 2/1991  | Hasegawa et al.              |
| 5,066,560 A       | 11/1991 | Tan et al.                   |
| 5,418,108 A       | 5/1995  | Kmiecik-Lawrynowicz et al.   |
| 5,827,633 A       | 10/1998 | Ong et al. .... 430/137      |
| 5,902,710 A *     | 5/1999  | Ong et al. .... 430/108.1    |
| 6,137,977 A *     | 10/2000 | Okado et al. .... 399/252    |
| 2002/0187415 A1   | 12/2002 | Jiang et al. .... 430/137.14 |
| 2002/0187416 A1 * | 12/2002 | Jiang et al. .... 430/137.14 |
| 2004/0152007 A1   | 8/2004  | Combes et al. .... 430/120   |
| 2006/0204876 A1 * | 9/2006  | Kaburagi et al. .... 430/105 |

2009/0269690 A1 \* 10/2009 Morris et al. .... 430/105

FOREIGN PATENT DOCUMENTS

|    |             |         |
|----|-------------|---------|
| EP | 0952493     | 10/1999 |
| WO | WO 98/50828 | 11/1998 |
| WO | WO 99/50714 | 10/1999 |

\* cited by examiner

Primary Examiner—Hoa V Le

(74) Attorney, Agent, or Firm—Morgan Lewis & Bockius LLP

(57) **ABSTRACT**

The invention provides a process for the manufacture of a toner which comprises the steps of:

- providing a latex dispersion containing primary resin particles and surfactant;
- providing a colorant dispersion containing primary colorant particles and surfactant;
- optionally providing a wax dispersion containing primary wax particles and surfactant;
- providing at least one carboxy functional compound of Formula (1), which may be in acid, salt and/or complex form:



wherein R is a carbocyclic or heterocyclic radical which may be optionally substituted and Z<sub>1</sub> is a bond or linker group and wherein the amount of carboxy functional compound of Formula (1) provided is greater than 3% by weight, the amount of carboxy functional compound being calculated according to the following equation:

amount of carboxy functional compound (% weight) =

$$\frac{100 \times \text{weight of carboxy functional compound}}{(\text{weight of carboxy functional compound} + \text{weight of solids content of latex, colorant and optional wax dispersions} + \text{weight of any additional surfactant})}$$

- mixing the latex dispersion, colorant dispersion, optional wax dispersion and said carboxy functional compound; and
- causing the particles in the mixture to associate.

The process advantageously may produce a toner of small size and narrow particle size distribution. The present invention also provides a toner manufactured by the process.

**15 Claims, No Drawings**

**TONER AND MANUFACTURING PROCESS  
THEREFOR**

This invention relates to toners for use in the formation of electrostatic images and processes for their manufacture.

Dry toners for development of an electrostatic image comprise small colored resin particles typically less than 50  $\mu\text{m}$  in size. The particle size distribution of the toner particles in a toner affects the quality of the final image. Ideally, a toner should be capable of forming an image with high resolution and high image density. Furthermore, the toner should preferably not suffer from problems such as filming which may be related, at least in part, to the particle size distribution.

Toners are conventionally produced by melt kneading of a pigment, resin and other toner ingredients, followed by milling or pulverisation to produce toner sized particles. Classification is then needed to generate an acceptably narrow particle size distribution of the toner particles.

More recently, attention has been focussed on chemical routes to toners, where a suitable particle size is not attained by a milling process, which thereby avoids the need for a classification step. By avoiding the classification step, less material is wasted and higher yields of toner can be attained, especially as the target particle size is reduced. Lower particle size toners are of considerable interest for a number of reasons, including better print resolution, lower pile height, greater yield from a toner cartridge, faster or lower temperature fusing, and lower paper curl.

Several chemical routes to toners have been exemplified in the prior art. These include suspension polymerisation, solution-dispersion processes and so-called aggregation processes. Several aggregation processes are known, for example, as described in U.S. Pat. Nos. 4,996,127, 5,418,108, 5,066,560 and 4,983,488, WO 98/50828 and WO 99/50714.

However, it is still desirable to provide further methods for making toners which are capable of reliably forming toner having a narrow particle size distribution.

According to one aspect of the present invention, there is provided a process for the manufacture of a toner which comprises the steps of:

- a) providing a latex dispersion containing primary resin particles and surfactant;
- b) providing a colorant dispersion containing primary colorant particles and surfactant;
- c) optionally providing a wax dispersion containing primary wax particles and surfactant;
- d) providing at least one carboxy functional compound of Formula (1), which may be in acid, salt and/or complex form:

Formula (1)



wherein R is a carbocyclic or heterocyclic radical which may be optionally substituted and Z<sub>1</sub> is a bond or linker group and wherein the amount of carboxy functional compound of Formula (1) provided is greater than 3% by weight, the amount of carboxy functional compound being calculated according to the following equation:

amount of carboxy functional compound (% weight) =

$$\frac{100 \times \text{weight of carboxy functional compound}}{(\text{weight of carboxy functional compound} + \text{weight of solids content of latex, colorant and optional wax dispersions} + \text{weight of any additional surfactant})}$$

e) mixing the latex dispersion, colorant dispersion, optional wax dispersion and said carboxy functional compound; and

f) causing the particles in the mixture to associate.

The present invention, in another aspect, provides a toner manufactured by the process.

Advantageously, the process according to the present invention has been found to provide a manufacturing route to toners which is capable of producing toners of narrow particle size distribution. In particular, the proportion of fine particles and the proportion of coarse particles (grit) may be reduced compared to an aggregation process in which the carboxy functional compound of Formula (1) (hereinafter "the carboxy functional compound") is not employed in the manner according to the present invention.

At the same time as providing a narrow particle size distribution, the process according to the present invention may satisfy many other requirements for a desirable process. The process may provide a great deal of control over the toner shape and, generally, no further treatment may be required to alter the shape. In particular, a shape may be provided, as desired, from substantially spherical to substantially irregular.

The process may be very efficient at incorporating a wax in the toner in order to improve its release properties as well as incorporating other components such as a charge control agent (CCA). The wax may be incorporated in the toner in relatively large amounts compared with some prior art processes and may be incorporated in uniformly sized wax domains, which may improve the transparency of prints formed by the toner.

The process can produce a toner which may be capable of one or more of the following: fixing to a substrate at low temperatures by means of heated fusion rollers; releasing from the fusion rollers over a wide range of fusion temperatures and speeds, and over a wide range of toner print densities; possessing good storage stability, print transparency, toner charging characteristics and does not lead to background development of the photoconductor; not leading to filming of the metering blade or development roller (for a mono-component device) or the carrier bead (for a dual-component device), or of the photoconductor; having high transfer efficiency from the photoconductor to the substrate or intermediate transfer belt or roller and from the transfer belt or roller (where used) to the substrate; enabling efficient cleaning of any residual toner remaining after image transfer where a mechanical cleaning device is used.

The carboxy functional compound may be provided in acid (i.e. protonated) form, in salt form, in complex form (as hereinafter defined) or a mixture of two or more of these forms. Accordingly, all the Formulae shown herein for the carboxy functional compound (including in the claims) encompass the compound in acid, salt and/or complex form, unless otherwise stated.

For the avoidance of doubt, the amount of the carboxy functional compound according to the equation above is an

amount calculated as a percentage (% by weight) of the total weight of the carboxy functional compound in all forms (i.e. acid, salt and/or complex), the solids content of the latex, colorant and optional wax dispersions (which includes both non-surfactant solids and surfactant) and any additional surfactant (i.e. surfactant other than that present in the latex, colorant and optional wax dispersions).

In Formula (1), R is a carbocyclic or heterocyclic radical, each of which may be optionally substituted. The term carbocyclic radical herein means a radical wherein the atoms linked to form the carbocyclic ring are all carbon atoms. The term heterocyclic radical herein means a radical wherein the atoms linked to form the heterocyclic ring comprise one or more heteroatoms selected from S, O and N.

The carbocyclic radical may be an aliphatic or aromatic radical. Examples of aromatic radical include phenyl or naphthyl. Examples of aliphatic radical include cycloalkyl (e.g. cyclohexyl), cycloalkenyl (e.g. cyclohexenyl) and cycloalkynyl (e.g. cyclohexynyl).

The heterocyclic radical may be a heteroaromatic radical. Examples of heteroaromatic ring radical include pyridinyl, diazinyl, triazinyl or quinolinyl. Other examples of heterocyclic radical include piperidinyl.

Preferably, R is an optionally substituted carbocyclic aromatic radical. More preferably, R is optionally substituted phenyl or naphthyl (including 1-naphthyl and 2-naphthyl, preferably 2-naphthyl), so that the carboxy functional compound may be represented thus:



Formula (1a)



Formula (1b)



Formula (1c)

wherein the phenyl or naphthyl groups of Formulae (1a)-(1c) may optionally be substituted with further substituents. Preferably, the carboxy functional compound is of Formula (1a) or (1b).

$Z_1$  is a bond (i.e. where the carboxy group is attached directly to R) or linker group.  $Z_1$  may be any known linker group.  $Z_1$  may, for example, be one of: —O—; an optionally substituted  $C_{1-20}$  (preferably  $C_{1-4}$ ) alkyl linker, e.g.  $-(CH_2)_x-$ ; an optionally substituted  $C_{1-20}$  (preferably  $C_{1-4}$ ) alkenyl linker; an optionally substituted  $C_{1-20}$  (preferably  $C_{1-4}$ ) alkoxy linker; or an optionally substituted  $C_{1-20}$  (preferably  $C_{1-4}$ ) polyether linker, e.g.  $-(OCH_2)_x-$  wherein x is an integer from 1 to 20 (preferably 1 to 4). Most preferably,  $Z_1$  is a bond. Thus, the Formulae (1a)-(1c) are preferably of Formulae (1a')-(1c'):



Formula (1a')



Formula (1b')



Formula (1c')

wherein the phenyl or naphthyl groups of Formulae (1a')-(1c') may optionally be substituted with further substituents.

The carboxy functional compound of Formula (1) may be provided as an acid (i.e. protonated form), as a salt, as a complex, or as a mixture of two or more of these. In preferred embodiments, the carboxy functional compound is substantially provided in salt form and/or complex form.

The salt form may be a salt of a metal species or non-metal species (e.g. ammonium ion). Preferably, the salt is a salt of a metal species. The metal species with which the carboxy functional compound may form a metal salt may be any suitable metal species, including any metal, metal oxide, metal hydroxide or metal halide. Preferably, the salt is a salt of a metal. In particular, the metal may comprise a group IA metal (e.g. lithium, sodium or potassium) or group IIA metal (e.g. magnesium or calcium), preferably a group IA metal.

In the salt form of the carboxy functional compound of Formula (1), the carboxy group, or groups if more than one, is preferably present in an ionic form, i.e.  $-CO_2^-M^+$  wherein  $M^+$  represents a metal ion or ammonium ion. Preferably  $M^+$  is selected from  $Li^+$ ,  $Na^+$ ,  $K^+$ ,  $Mg^+$ ,  $Ca^+$ , and  $NH_4^+$  (more preferably  $Li^+$ ,  $Na^+$ ,  $K^+$ , and  $NH_4^+$ ). For the avoidance of doubt, the term salt herein excludes a complex as hereinafter defined. Typically, therefore, the salt has a ratio of carboxy functional compound: metal of 1:1 or less (e.g. 1:2, such as where there are two or more carboxy groups in the compound). More typically, the salt has a ratio of carboxy functional compound: metal of 1:1.

The term complex herein means a metal complex wherein the ratio of carboxy functional compound: metal is 2:1 or higher (e.g. 3:1), preferably 2:1. The metal of the complex may be a transition metal (e.g. titanium, vanadium, chromium, manganese, iron, cobalt, nickel, copper or zinc) or a group IIIB metal (e.g. aluminium or gallium). Preferred metal species with which the carboxy functional compound may form a metal complex are selected from aluminium, chromium, manganese, iron, cobalt, nickel, copper or zinc (especially aluminium and chromium).

Preferably, the carboxy functional compound of Formula (1) further carries at least one additional ionisable group (i.e. in addition to the carboxy group in Formula (1)). More preferably, the additional ionisable group may also be capable of forming a salt or of coordinating to a metal species with which the compound may form a complex. Preferred additional ionisable groups include another COOH, OH, NH or SH and

most preferred is OH. Preferably, the additional ionisable group is carried on R. In other words, preferably R carries both the  $-Z_1-CO_2H$  group and the additional ionisable group (which is preferably OH). The additional ionisable group may be attached directly to R or via a linker group, which may be any known linker group including those examples of linker groups for  $Z_1$  described above.

In view of the above preferences, a preferred carboxy functional compound is of Formula (2):



Formula (2)

where  $Z_2$  is a bond or linker group and A is an ionisable group.

$Z_2$  is a bond (i.e. where A is attached directly to R) or linker group.  $Z_2$  may be any known linker group.  $Z_2$  may, for example, be one of: —O—; an optionally substituted  $C_{1-20}$  (preferably  $C_{1-4}$ ) alkyl linker, e.g.  $-(CH_2)_x-$ ; an optionally substituted  $C_{1-20}$  (preferably  $C_{1-4}$ ) alkenyl linker; an optionally substituted  $C_{1-20}$  (preferably  $C_{1-4}$ ) alkoxy linker; or an optionally substituted  $C_{1-20}$  (preferably  $C_{1-4}$ ) polyether linker, e.g.  $-(OCH_2)_x-$  wherein x is an integer from 1 to 20 (preferably 1 to 4). Most preferably,  $Z_2$  is a bond. Most preferably, both  $Z_1$  and  $Z_2$  are each a bond.

A is preferably an ionisable group selected from the group consisting of COOH, OH, NH<sub>2</sub> or SH and most preferably A is OH.

Most preferably, the  $-Z_1-CO_2H$  and  $-Z_2-A$  groups are attached to R at adjacent ring positions. This positioning may facilitate coordination of the  $CO_2H$  and A groups to the metal species with which the compound may form a complex. For instance, in the preferred embodiments where R is phenyl or naphthyl, preferably the carboxy functional compound has a Formula (3) or (4):



Formula (3)



Formula (4)

more preferably, a Formula (5) or (6):



Formula (5)

-continued

Formula (6)



10

and most preferably, a Formula (7) or (8):



Formula (7)



Formula (8)

15

wherein in Formulae (3)-(8) the phenyl or naphthyl groups may optionally be substituted with further substituents.

The optional substituents for R (including for the phenyl and naphthyl groups of Formulae (1a)-(1c) and (3)-(8)),  $Z_1$  and  $Z_2$  are preferably selected from the following list: optionally substituted alkyl (especially optionally substituted  $C_{1-4}$  alkyl), optionally substituted cycloalkyl, optionally substituted alkoxy (especially optionally substituted  $C_{1-4}$  alkoxy), optionally substituted aryl, optionally substituted heteroaryl, optionally substituted aryloxy, optionally substituted amino, hydroxyl, halo, cyano, nitro, silyl, silyloxy, azo, sulpho (i.e. SO<sub>3</sub>H), phosphato (i.e. PO<sub>3</sub>H<sub>2</sub>), —COOR<sup>1</sup>, —OCOOR<sup>1</sup>, —OCOR<sup>1</sup>, —COR<sup>1</sup>, —CONR<sup>1</sup>R<sup>2</sup>, —OCONR<sup>1</sup>R<sup>2</sup>, —SR<sup>1</sup>, —SO<sub>2</sub>NR<sup>1</sup>R<sup>2</sup>, or —SO<sub>2</sub>R<sup>1</sup>, wherein R<sup>1</sup> and R<sup>2</sup> each independently represent H, optionally substituted alkyl, optionally substituted cycloalkyl, or optionally substituted aryl. When any substituent group from the foregoing list is itself described as being optionally substituted, it may be substituted with any of the substituents from the same list. Groups such as sulpho, phosphato and carboxy (i.e. COOH) may be present in a salt form. It will be appreciated from the foregoing list that, in addition to the  $-Z_1-CO_2H$  and  $-Z_2-A$  groups, R may be substituted still further by additional  $-CO_2H$  or A groups. A preferred optional substituent for R is optionally substituted alkyl (especially  $C_{1-4}$  alkyl), e.g. methyl, ethyl, propyl, isopropyl, n-butyl and tert-butyl. Preferably, any substituent on R does not comprise more than 6 carbon atoms and more preferably does not comprise more than 4 carbon atoms.

Preferred examples of the carboxy functional compound suitable for use in the present invention include the following (and their salts and complexes):

- 60     salicylic acid;
- substituted salicylic acids;
- alkyl substituted salicylic acids (e.g. di-tertbutylsalicylic acid);
- 65     naphthoic acid;
- substituted naphthoic acids;
- alkyl substituted naphthoic acids;

hydroxy naphthoic acids, especially 2-hydroxy-3-naphthoic acids (e.g. "bon acid");

substituted hydroxy naphthoic acids, especially substituted 2-hydroxy-3-naphthoic acids;

alkyl substituted hydroxy naphthoic acids, especially alkyl substituted 2-hydroxy-3-naphthoic acids.

More preferred examples among these include optionally substituted salicylic acids, especially alkyl substituted salicylic acids (e.g. di-tertbutylsalicylic acid) and optionally substituted hydroxy naphthoic acids, especially optionally substituted 2-hydroxy-3-naphthoic acids (e.g. "bon acid"). In more preferred embodiments, the invention employs a salt and/or complex of these examples of carboxy functional compound. Commercial products include Bontron<sup>TM</sup> E81, E82, E84 and E88 (Orient Chem. Co.) and LR 147 (Japan Carlit).

There may be provided a mixture of two or more of the carboxy functional compounds. In that case, it is the total amount of all the carboxy functional compounds used which should be greater than 3% by weight. Preferred combinations of the carboxy functional compounds include a mixture of an optionally substituted salicylic acid (e.g. di-tertbutylsalicylic acid) and an optionally substituted hydroxy naphthoic acid, especially an optionally substituted 2-hydroxy-3-naphthoic acid (e.g. bon acid), either or both of which preferably may be provided in salt and/or complex form. Especially preferred combinations include a combination of an optionally substituted salicylic acid in complex form and an optionally substituted hydroxy naphthoic acid in salt form.

As described above, the carboxy functional compound may be provided as the acid form compound (i.e. protonated form), as a salt of the compound, as a complex, or as a mixture of two or more of these. Preferably, at least a portion of the carboxy functional compound is present in the form of a salt or complex. Preferably, a salt and/or complex, especially a complex, form of the carboxy functional compound is present in an amount of at least 1% by weight, more preferably greater than 2% by weight and most preferably greater than 3% by weight. For instance, a salt and/or complex, especially a complex, form of the carboxy functional compound may be present in an amount of 1 to 4% by weight.

Preferably, the amount of carboxy functional compound provided is not more than 10%, more preferably not more than 7% and most preferably not more than 5%, by weight. Accordingly, a preferred range for the total amount of carboxy functional compound (i.e. in all forms) is 3 to 10%, a more preferred range is 3 to 7% and a most preferred range is 3 to 5%.

All or at least a portion of the carboxy functional compound may be milled with the colorant, so as to form part of the colorant dispersion. Alternatively or additionally, at least a portion of the carboxy functional compound may be provided separately before mixing with the dispersions in the mixing step. Preferably, at least a portion, more preferably all, of the carboxy functional compound is provided separately. Where at least a portion of the carboxy functional compound is provided separately it may be provided, for example, as a wet-cake or solution. The wet-cake or solution may be a wet-cake or solution of the carboxy functional compound in salt or complex form. Where at least a portion of the carboxy functional compound is provided separately it is preferably provided as a wet cake. The solids content of the wet cake or solution is preferably at least 10% by weight. Where the carboxy functional compound is provided separately it is then mixed with the dispersions in the mixing step (e).

Preferably, additional surfactant (i.e. additional to the surfactant present as part of the latex, colorant and optional wax dispersions) is provided. Although preferable, the additional

surfactant is, however, optional and not essential. The process preferably comprises mixing the additional surfactant with the latex dispersion, colorant dispersion, optional wax dispersion and carboxy functional compound in step (e). The additional surfactant may be provided with the carboxy functional compound (e.g. as part of a wet-cake) or provided separately. Preferably, the additional surfactant is an ionic surfactant, more preferably an ionic surfactant with a charge of the same sign as the surfactants used to stabilise the latex, colorant and optional wax dispersions and most preferably the same ionic surfactant as the surfactants used to stabilise the latex, colorant and optional wax dispersions. This is particularly preferable where a pH switch process is used to cause the particle association in step (f). The amount of the additional surfactant provided is preferably in the range 0.1 to 10% (more preferably 0.5 to 5%) by weight based on the total weight of the carboxy functional compound, the solids content of the latex, colorant and optional wax dispersions and surfactant (namely the additional surfactant).

20 The latex dispersion contains primary resin particles which are particles of the binder resin which goes to make up the bulk of the toner.

Preferably, the latex dispersion is a dispersion of the resin particles in water. The latex dispersion preferably comprises an ionic surfactant to stabilise the resin particles in dispersion. Optionally, a non-ionic surfactant may also be incorporated into the latex dispersion.

In this invention, examples of anionic surfactants are:

30 Alkyl aryl sulphonates (e.g. sodium dodecylbenzenesulphonate)

Alkyl sulphates

Alkyl ether sulphates

Sulphosuccinates

Phosphate esters

35 Alkyl carboxylates

Alkyl ethoxylate carboxylates

Alkyl propoxylate carboxylates;

Examples of cationic surfactants are:

Quaternary ammonium salts

Benzalkonium chloride

Ethoxylated amines;

Examples of non-ionic surfactants are:

Alkyl ethoxylates

Alkyl propoxylates

Alkyl aryl ethoxylates

Alkyl aryl propoxylates

Ethylene oxide/propylene oxide copolymers.

In one preferred form of the process according to the present invention, the association in step (f) is caused by a pH switch process. Thus, the ionic surfactant present in the latex dispersion contains a group which can be converted from an ionic to a non-ionic form (and vice versa) by adjustment of pH. Preferred such groups include carboxylic acid or tertiary amine groups. Further preferably in that same preferred form of the process, the ionic surfactant on the latex dispersion has a charge (i.e. anionic or cationic) of the same sign as that of the ionic surfactant used in the colorant dispersion and optional wax dispersion described below. It is further preferred in such a case to use the same surfactant for each of the individual dispersions. This enables the association step (f) of the process to be performed by changing the pH in order to change the charge on the surfactant and thereby destabilise the dispersions and so cause association. Such a process is described fully in the applicant's earlier patent applications published as WO 98/50828 and WO 99/50714, the full contents of which are incorporated herein. In the foregoing preferred pH switch form of the process according to the present

invention, the individual components can be particularly well mixed prior to inducing association, which, in turn, may lead to improved homogeneity of distribution of the components in the final toner. The pH switch embodiment furthermore may not require the addition of large quantities of salt or surfactant to induce association.

The latex dispersion may be prepared by polymerisation processes known in the art, preferably by emulsion polymerisation.

The molecular weight of the latex can be controlled by use of a chain transfer agent (e.g. a mercaptan), by control of initiator concentration and/or by heating time.

The latex dispersion may comprise a single latex or may comprise a combination of two or more separate latexes.

The latex(es) may be monomodal or bimodal in their molecular weight distribution. In one preferred embodiment, at least one latex with monomodal molecular weight distribution is combined with at least one latex with bimodal molecular weight distribution. By a latex with a monomodal molecular weight distribution is meant one in which the gpc spectrum shows only one peak. By a latex with a bimodal molecular weight distribution is meant one where the gpc spectrum shows two peaks, or a peak and a shoulder.

It is preferred that the overall molecular weight distribution of all the resin in the latex dispersion (i.e. the overall molecular weight distribution of the resin in the toner) shows  $M_w/M_n$  of 3 or more, more preferably 5 or more, most preferably 10 or more. The  $T_g$  of each resin is preferably from 30 to 100°C., more preferably from 45 to 75°C., most preferably from 50 to 70°C. If the  $T_g$  is too low, the storage stability of the toner will be reduced. If the  $T_g$  is too high, the melt viscosity of the resin will be raised, which will increase the fixation temperature and the temperature required to achieve adequate transparency. It is preferred that all the components in the resin have a substantially similar  $T_g$ .

The latex may comprise resin particles made from one or more of the following preferred monomers for emulsion polymerisation: styrene and substituted styrenes; acrylate and methacrylate alkyl esters (e.g. butyl acrylate, butyl methacrylate, methyl acrylate, methyl methacrylate, ethyl acrylate or methacrylate, octyl acrylate or methacrylate, dodecyl acrylate or methacrylate etc.); acrylate or methacrylate esters with polar functionality, for example hydroxy or carboxylic acid functionality, hydroxy functionality being preferred (particularly 2-hydroxyethyl acrylate, 2-hydroxyethyl methacrylate, or hydroxy-terminated poly(ethylene oxide) acrylates or methacrylates, or hydroxy-terminated poly(propylene oxide) acrylates or methacrylates), examples of monomers with carboxylic acid functionality including acrylic acid and beta-carboxyethylacrylate; vinyl type monomers such as ethylene, propylene, butylene, isoprene and butadiene; vinyl esters such as vinyl acetate; other monomers such as acrylonitrile, maleic anhydride, vinyl ethers. The resin may comprise a co-polymer of two or more of the above monomers.

Preferred latexes comprise resin particles which are made from copolymers of (i) a styrene or substituted styrene, (ii) at least one alkyl acrylate or methacrylate and (iii) an hydroxy-functional acrylate or methacrylate.

The latex dispersion may comprise the following, not used in emulsion polymerisation: a dispersions of polyester, poly-urethane, hydrocarbon polymer, silicone polymer, polyamide, epoxy resin and other resin known in the art.

The average size of the primary resin particles in the latex dispersion, as measured using photon correlation spectroscopy, is preferably less than 200 nm and more preferably less than 150 nm. The average size of the primary resin particles may, for example lie in the range 80-120 nm.

Preferably, the colorant dispersion is a dispersion in water. The colorant dispersion may be prepared by processes known in the art, preferably by milling the colorant with a surfactant in an aqueous medium.

Alternatively, an aqueous dispersion of colorant particles may be produced by a solution dispersion process in the following way. A polymer (e.g. polyester) is dissolved in an organic solvent. Preferably the solvent used should be immiscible with water, dissolve the polymer and/or be removable by distillation relatively easily. Suitable solvents comprise xylene, ethyl acetate and/or methylene chloride. To this solution is added a colorant, either a pigment or a dye. If a dye is used this is simply dissolved in the polymer solution to produce a colored liquid solution. If a pigment is used it may be added, preferably with one or more suitable pigment dispersants (which may be ionic or non-ionic). The colored polymer solution is then dispersed in water with a surfactant and the solvent removed by distillation to leave an aqueous dispersion of pigmentary particles containing the colorant dissolved or dispersed within the polymer.

The colorant dispersion preferably comprises an ionic surfactant to stabilise the colorant particles in dispersion. Optionally, a non-ionic surfactant may also be incorporated into the colorant dispersion. Examples of ionic and non-ionic surfactants for the colorant dispersion are the same as for the latex dispersion described above.

In one preferred embodiment of the process wherein the association is caused by a pH switch process, the colorant dispersion is stabilised with an ionic surfactant, which has the same sign as the ionic surfactant used for the latex dispersion and the optional wax dispersion and which is capable of being converted from an ionic to a non-ionic form (and vice versa) by a change in pH.

The colorant may be any color including black. The colorant contained in the colorant dispersion may comprise a pigment or a dye. Preferably, the colorant comprises a pigment. Any suitable pigment known in the art can be used, including black and magnetic pigments, for example carbon black, magnetite, copper phthalocyanine, quinacridones, xanthanes, mono- and dis-azo pigments, naphthols etc. Other examples include CI Pigment Blue 15:3, CI Pigment Red 31, 57, 81, 122, 146, 147, 184 or 185; CI Pigment Yellow 12, 13, 17, 74, 155 180 or 185. In full colour printing it is normal to use yellow, magenta, cyan and black toners. However it is possible to make specific toners for spot colour or custom colour applications. The colorant is preferably present in an amount from 1-15% by weight based on the total weight of the carboxy functional compound, the solids content of the latex, colorant and optional wax dispersions (including surfactant therein) and any additional surfactant, more preferably from 1.5-10% by weight, most preferably from 2-8% by weight. These ranges are most applicable for organic, non-magnetic pigments. If, for example, magnetite was used as a magnetic filler/pigment, the level would typically be higher.

Preferably, in one embodiment of the process, the colorant dispersion is prepared by milling the colorant with an ionic surfactant, and optionally a non-ionic surfactant, until the particle size is suitably reduced.

Preferably, the volume average size of the primary colorant particle, which may be measured by a light scattering method, is less than 300 nm, more preferably less than 200 nm and most preferably less than 100 nm.

Preferably, a wax dispersion is used in the process. The wax dispersion is preferably a dispersion in water. The wax dispersion is preferably prepared by the mixing together of a wax with an ionic surfactant to stabilise the wax particles in dispersion. Examples of ionic and optionally non-ionic surfac-

## 11

tants for the wax dispersion are the same as for the latex and colorant dispersions described above.

In one preferred embodiment of the process wherein the association is caused by a pH switch process, the wax dispersion is stabilised with an ionic surfactant, which has the same sign as the ionic surfactant used for the latex dispersion and the colorant dispersion and which is capable of being converted from an ionic to a non-ionic form (and vice versa) by a change in pH.

The wax should have a melting point (mpt) (as measured by the peak position by differential scanning calorimetry (dsc)) of from 50 to 150° C., preferably from 50 to 130° C., more preferably from 50 to 110° C., especially from 65 to 85° C. If the mpt is >150° C. the release properties at lower temperatures are inferior, especially where high print densities are used. If the mpt is <50° C. the storage stability of the toner will suffer, and the toner may be more prone to showing filming of the OPC or metering blade.

The wax may comprise any conventionally used wax. Examples include hydrocarbon waxes (e.g. polyethylenes such as Polywax™ 400, 500, 600, 655, 725, 850, 1000, 2000 and 3000 from Baker Petrolite; paraffin waxes and waxes made from CO and H<sub>2</sub>, especially Fischer-Tropsch waxes such as Paraflint™ C80 and H1 from Sasol; ester waxes, including natural waxes such as Carnauba and Montan waxes; amide waxes; and mixtures of these. Hydrocarbon waxes are preferred, especially Fischer-Tropsch, paraffin and polyethylene waxes. It is especially preferred to use a mixture of Fischer-Tropsch and Carnauba waxes, or a mixture of paraffin and Carnauba waxes.

The amount of wax used in the process is preferably from 1 to 30% by weight based on the total weight of the carboxy functional compound, the solids content of the latex, colorant and wax dispersions and surfactant, more preferably from 3 to 20% by weight, especially from 5 to 15% by weight. If the level of wax is too low, the release properties may be inadequate for oil-less fusion. Too high a level of wax will reduce storage stability and lead to filming problems. The distribution of the wax through the toner is also an important factor, it being preferred that wax is substantially not present at the surface of the toner.

The volume average particle size of the primary wax particles, which may be measured by a light scattering method, in the dispersion is preferably in the range from 100 nm to 2 µm, more preferably from 100 to 800 nm, still more preferably from 150 to 600 nm, and especially from 200 to 500 nm. The wax particle size is chosen such that an even and consistent incorporation into the toner is achieved.

Within the scope of the invention and claims, in embodiments, the latex dispersion, colorant dispersion and optional wax dispersion are separate dispersions which are then mixed (in step (e)). However, in certain embodiments, the primary resin particles may be prepared in a dispersion along with either or both of the primary colorant and/or wax particles, such that the latex, colorant and/or wax dispersions may be one and the same. It is also possible that the primary colorant and wax particles are prepared in one dispersion so that the colorant and wax dispersions are one and the same.

The process of the present invention may further comprise providing a charge control agent (CCA) which may be selected from such known classes of CCAs as metal azo complexes, phenolic polymers and calixarenes, nigrone, quaternary ammonium salts, and arylsulphones. Preferred CCAs are colourless.

The CCA may be provided as a component of one of the dispersion in steps (a)-(c) or the CCA may be provided separately and added as part of the pre-association mixture, pref-

## 12

erably as a solution or wet cake. Additionally or alternatively, a CCA may be added externally to the toner prepared by the process, in which case a suitable high-speed blender may be used, e.g. a Nara Hybridiser or Henschel blender. Where the CCA is added externally it is preferably added to the dried toner.

Preferably, each dispersion is a dispersion in water.

Mixing of the dispersions in step (e) may be performed by any conventional method of mixing dispersions. The mixing may include a low shear condition (e.g. using a low shear stirring means) and/or a high shear condition (e.g. using a rotor-stator type mixer). The mixed dispersions may be heated at a temperature below the Tg prior to association.

The particles in the mixture obtained in step (e) may be caused to associate in step (f) by any suitable method known in the art. For instance, the association may be caused by heating and stirring as described, for example, in U.S. Pat. No. 4,996,127 (Nippon Carbide), by the addition of an inorganic salt as described, for example, in U.S. Pat. No. 4,983,488 (Hitachi Chemical Co.) or by the action of organic coagulants, including counterionic surfactants as described, for example, in U.S. Pat. No. 5,418,108 and numerous other patents of Xerox.

In a preferred method, the association is caused by a pH switch, i.e. by effecting a change in the pH, preferably either from a basic pH to an acidic pH or from an acidic pH to a basic pH. Such association processes are described in WO 98/50828 and WO 99/50714. In this case, surfactant present in each of the dispersions is reversibly ionisable or de-ionisable, i.e. contains a group which can be converted from an ionic to a non-ionic form and vice versa by adjustment of pH. In a particularly preferred example, the surfactant may contain a carboxylic acid group, and the dispersions may be mixed at neutral to high (i.e. above neutral) pH with association then being effected by addition of an acid, which decreases the pH and converts the surfactant from its dispersion stabilising anionic form to its non-stabilising non-ionic form. Alternatively, in another preferred example, the surfactant may contain a group which is the acid salt of a tertiary amine, and the dispersions may be mixed at neutral to low (i.e. below neutral) pH with association then being effected by addition of a base which increases the pH and converts the surfactant from its dispersion stabilising cationic form to its non-stabilising non-ionic form. The pH switch processes allow a very efficient use of surfactant and have the ability to keep overall surfactant levels very low. This is advantageous since residual surfactant in the final toner can be problematic, especially in affecting the charging properties of the toner, particularly at high humidity. In addition, such processes avoid the need for large quantities of salt, as required for some prior art processes, which would need to be washed out.

Stirring and mixing are preferably performed during the association step.

The association step is preferably carried out below the Tg of the resin in the latex.

After the association step (f), the process preferably comprises a further step (g) of heating and/or stirring the associated mixture (preferably at a temperature below the Tg of the resin particles). Preferably such heating and/or stirring of the associated mixture causes loose aggregates to form. The aggregates are composite particles comprising the primary particles of resin, colorant and optionally wax. Preferably, the aggregates are of particle size from 1 to 20 µm, more preferably from 2 to 20 µm. Once the desired aggregate particle size is established, the aggregates may be stabilised against further growth. This may be achieved, for example, by addition of further surfactant, and/or by a change in pH where a pH

## 13

switch process was employed for the association as is known in the art (e.g. WO 98/50828).

After the association step (f) and optional further step (g) of heating and/or stirring to establish the desired particle size, the temperature may then be raised above the  $T_g$  of the resin in a step (h) to form toner particles. The step (h) brings about coalescence of the particles, e.g. within each aggregate and/or between aggregates, to form toner particles. The toner particles typically have a volume average particle size from 2 to 20  $\mu\text{m}$ , more preferably 4 to 10  $\mu\text{m}$ , still more preferably 5 to 9  $\mu\text{m}$  and most preferably 6 to 8  $\mu\text{m}$ . During this step of heating above the  $T_g$  the shape of the toner may be controlled through selection of the temperature and the heating time.

The dispersion of toner particles may then be cooled and the toner particles recovered, e.g. by filtration, for subsequent use as an electrophotographic toner. The toner may then optionally be washed (e.g. to remove at least some surfactant) and/or optionally be dried using methods known in the art. The washing step, for example, may comprise washing with water, or dilute acid or base. The washing step typically removes at least some (preferably most) of any portion of the carboxy functional compound which is present in a protonated form or in the form of a salt. Thus, carboxy functional compound not in the form of a metal complex may be utilised in the process to assist formation of a toner having narrow particle size distribution whilst substantially not remaining in the final toner after a washing step.

The toner particles, especially the recovered and dried toner particles, may be blended with one or more surface additives to improve the powder flow properties of the toner, or to tune the tribocharge properties, as is known in the art. Typical surface additives include, but are not limited to, silica, metal oxides such as titania and alumina, polymeric beads (for example acrylic or fluoropolymer beads) and metal stearates (for example zinc stearate). Conducting additive particles may also be used, including those based on tin oxide (e.g. those containing antimony tin oxide or indium tin oxide).

Each surface additive may be used at 0.1-5.0 wt % based on the weight of the unblended toner (i.e. the toner prior to addition of the surface additive), preferably 0.2-3.0 wt %, more preferably 0.25-2.0 wt %. The total level of surface additives used may be from about 0.1 to about 10 wt %, preferably from about 0.5 to 5%, based on the weight of the unblended toner.

The additives may be added by blending with the toner, using, for example, a Henschel blender, a Nara Hybridiser, or a Cyclomix blender (Hosokawa).

The particles of the above surface additives, including silica, titania and alumina, may be made hydrophobic, e.g. by reaction with a silane and/or a silicone polymer. Examples of hydrophobising groups include alkyl halosilanes, aryl halosilanes, alkyl alkoxy silanes (e.g. butyl trimethoxysilane, isobutyl trimethoxysilane and octyl trimethoxysilane), aryl alkoxy silanes, hexamethyldisilazane, dimethylpolysiloxane and octamethylcyclotetrasiloxane. Other hydrophobising groups include those containing amine or ammonium groups. Mixtures of hydrophobising groups can be used (for example mixtures of silicone and silane groups, or alkylsilanes and aminoalkylsilanes.)

Examples of hydrophobic silicas include those commercially available from Nippon Aerosil, Degussa, Wacker-Chemie and Cabot Corporation. Specific examples include those made by reaction with dimethyldichlorosilane (e.g. Aerosil™ R972, R974 and R976 from Degussa); those made by reaction with dimethylpolysiloxane (e.g. Aerosil™ RY50, NY50, RY200, RY200S and R202 from Degussa); those made by

## 14

reaction with hexamethyldisilazane (e.g. Aerosil™ RX50, NAX50, RX200, RX300, R812 and R812S from Degussa); those made by reaction with alkylsilanes (e.g. Aerosil™ R805 and R816 from Degussa) and those made by reaction with octamethylcyclotetrasiloxane (e.g. Aerosil™ R104 and R106 from Degussa).

The primary particle size of suitable surface additives, especially silicas, is typically from 5 to 200 nm, preferably from 7 to 50 nm. The BET surface area of the additives, especially silicas, may be from 10 to 350  $\text{m}^2/\text{g}$ , preferably 30-300  $\text{m}^2/\text{g}$ . Combinations of additives, especially silicas, with different particle size and/or surface area may be used.

It is possible to blend the different size additives in a single blending step, but it is often preferred to blend them in separate blending steps. In this case, the larger additive may be blended before or after the smaller additive. It may further be preferred to use two stages of blending, where in at least one stage a mixture of additives of different particle size is used. For example, an additive with low particle size may be used in the first stage, with a mixture of additives of different particle size in the second step.

Where titania is used, it is preferred to use a grade which has been hydrophobised, e.g. by reaction with an alkylsilane and/or a silicone polymer. The titania may be crystalline or amorphous. Where crystalline it may consist of rutile or anatase structures, or mixtures of the two. Examples include grades T805 or NKT90 from Nippon Aerosil and STT-30A from Titan Kogyo.

Hydrophilic or hydrophobic grades of alumina may be used. An example is Aluminium Oxide C from Degussa.

It is often preferred to use combinations of silica and titania, or of silica, titania and alumina. Combinations of large and small silicas, as described above, can be used in conjunction with titania, alumina, or with blends of titania and alumina. It is also often preferred to use silica alone. In that case, combinations of large and small silicas, as described above, can be used.

Preferred formulations of surface additives include those in the following list:

hydrophobised silica;  
large and small particle size silica combinations, which silicas may be optionally hydrophobised;  
hydrophobised silica and one or both of hydrophobised titania and hydrophilic or hydrophobised alumina;  
large and small particle size silica combinations as described above; and  
one or both of hydrophobised titania and hydrophilic or hydrophobised alumina.

Polymer beads or zinc stearate may be used to improve the transfer efficiency or cleaning efficiency of the toners. Charge control agents (CCAs) may be added in the external formulation (i.e. surface additive formulation) to modify the charge level or charging rate of the toners.

The process according to the present invention is especially suitable for producing a toner of narrow particle size distribution.

According to a further aspect of the present invention there is provided a toner obtainable by the process of the present invention wherein the volume average particle size of the toner is in the range from 2 to 20  $\mu\text{m}$  and the  $\text{GSD}_{\text{v}}$  value is not greater than 1.30.

The volume average particle size of the toner is preferably in the range from 4 to 10  $\mu\text{m}$ , more preferably 5 to 9  $\mu\text{m}$ , and most preferably in the range from 6 to 8  $\mu\text{m}$ . The volume average particle size and the particle size distribution as defined hereinafter ( $\text{GSD}_{\text{v}}$  and  $\text{GSD}_{\text{d}}$ ) refer to sizes as measured using a Coulter™ counter with a 100  $\mu\text{m}$  aperture.

## 15

Although it will be appreciated that other methods of preparing the toner for obtaining the Coulter™ counter measurement can be used, for example as described in U.S. Pat. No. 4,985,327, the Coulter™ counter measurement may be conveniently obtained in the present invention by analysing the dispersion of toner particles produced after the coalescence step of the process.

The GSD<sub>n</sub> value is defined by the following expression:

$$GSD_n = D_{50}/D_{15.9}$$

wherein D<sub>50</sub> is the particle size below which 50% by number of the toner particles have their size and D<sub>15.9</sub> is the particle size below which 15.9% by number of the toner particles have their size.

Preferably, the GSD<sub>n</sub> value is not greater than 1.28 and more preferably not greater than 1.25.

A GSD<sub>v</sub> value is defined by the following expression:

$$GSD_v = D_{84.1}/D_{50}$$

wherein D<sub>84.1</sub> is the particle size below which 84.1% by volume of the toner particles have their size and D<sub>50</sub> is the particle size below which 50% by volume of the toner particles have their size.

Preferably the GSD<sub>v</sub> value is not greater than 1.30, more preferably not greater than 1.25, still more preferably not greater than 1.23 and most preferably not greater than 1.20.

The GSD<sub>n</sub> and GSD<sub>v</sub> values of the toner of the present invention are calculated from the particle size distribution obtained by a Coulter™ Counter using a 100 µm aperture as described above. For example, a Coulter™ Multisizer II instrument may be used.

The low GSD<sub>n</sub> and GSD<sub>v</sub> of the toner according to the present invention provides, among other things, that the toner may possess a more uniform charge distribution leading to improved image quality and have a lower tendency toward filming.

The toner according to the present invention preferably has a mean circularity, as hereinafter defined, of the toner particles as measured by a Flow Particle Image Analyser of at least 0.90, more preferably at least 0.93.

Further preferably, the shape factor of the toner particles, SF1, as hereinafter defined, is at most 165, more preferably at most 155.

Additionally preferably, the shape factor of the toner particles, SF2, as hereinafter defined, is at most 155, more preferably at most 145.

The smoothness of the toner after the coalescence stage may also be assessed by measuring the surface area of the toner, for example by the BET method. It is preferred that the BET surface area of the unblended toner is in the range 0.5-1.5 m<sup>2</sup>/g.

Toner having the above shape properties has been found to have high transfer efficiency from the photoconductor to a substrate (or to an intermediate transfer belt or roller), in some cases close to 100% transfer efficiency.

The shape of the toner may be measured by use of a Flow Particle Image Analyser (Sysmex FPIA) and by image analysis of images generated by scanning electron microscopy (SEM).

The circularity is defined as the ratio:

$$L_o/L$$

where L<sub>o</sub> is the circumference of a circle of equivalent area to the particle, and L is the perimeter of the particle itself.

## 16

The shape factor, SF1, is defined as:

$$SF1 = (ML)^2/A \times \pi/4 \times 100, \text{ where } ML = \text{maximum length across toner, } A = \text{projected area}$$

5 The shape factor, SF2, is defined as:

$$SF2 = P^2/A \times 1/4\pi \times 100, \text{ where } P = \text{the perimeter of the toner particle, } A = \text{projected area}$$

An average of approximately 100 particles is taken to 10 define the shape factors (SF1 and SF2) for the toner.

If the toner is designed for a printer or copier which does not employ a mechanical cleaning device, it may be preferred to coalesce the toner until a substantially spherical shape is attained, e.g. wherein the mean circularity is at least 0.98. If, however, the toner is designed for use in a printer or copier in which a mechanical cleaning device is employed to remove residual toner from the photoconductor after image transfer, it may be preferred to select a smooth but off-spherical shape, 15 where the mean circularity is in the range 0.90-0.99, preferably 0.93-0.98, more preferably 0.94-0.98 and still more preferably 0.94-0.96, where SF1 is 105-165, preferably 105-155, more preferably 105-150 and still more preferably 105-145 and where SF2 is 105-155, preferably 105-145, more preferably 105-140 and still more preferably 105-135. In the smooth but off-spherical shape, the SF1 is particularly preferably 130-150 and most particularly preferred of all 135-145 and SF2 is particularly preferably 120-140, and most particularly preferred of all 125-135.

30 Where a wax is used in the process to obtain the toner, the wax is preferably present in the toner in domains of mean diameter 2 µm or less, preferably 1.5 µm or less. Preferably, the wax domains are of mean diameter 0.5 µm or greater. If the mean size of the wax domains is >2 µm, the transparency of the printed film may be reduced, and the storage stability may decrease. The domain size values are preferably those measured by analysing sections of the toner by transmission electron microscopy. Preferably the wax is not substantially 35 present at the surface of the toner.

40 The toner may be used as a mono-component or a dual component developer. In the latter case the toner is mixed with a suitable carrier bead.

45 Advantageously, the toner may be capable of fixing to the substrate at low temperatures by means of heated fusion rollers where no release oil is applied and may be capable of releasing from the fusion rollers over a wide range of fusion temperatures and speeds, and over a wide range of toner print densities. Furthermore, preferably, the toner according to the invention does not lead to background development of the photoconductor (OPC) and preferably does not lead to filming of the metering blade or development roller (for a mono-component device) or the carrier bead (for a dual-component device), or of the photoconductor.

50 Preferably, the haze values of prints using the toner of the invention do not vary considerably with fusion temperature. Haze may be assessed using a spectrophotometer, for example a Minolta CM-3600d, following ASTM D 1003. Preferably, the haze at a print density of 1.0 mg/cm<sup>2</sup> is below 60 40, preferably below 30, and the ratio of the values at fusion temperatures of 130 and 160° C. is preferably at most 1.5, more preferably 1.3 and most preferably 1.2.

The invention may be particularly suitable for use in an 65 electroreprographic apparatus or method where one or more of the following hardware conditions of an electroreprographic device applies:

17

- i) where the device contains a developer roller and metering blade (i.e. where the toner is a monocomponent toner);
- ii) where the device contains a cleaning device for mechanically removing waste toner from the photoconductor; 5
- iii) where the photoconductor is charged by a contact charging means;
- iv) where contact development takes place or a contact development member is present;
- v) where oil-less fusion rollers are used;
- vi) where the above devices are four colour printers or copiers, including tandem machines

Preferably, the invention provides a toner which satisfies many requirements simultaneously. The toner may be particularly advantageous for use in a mono-component electroreprographic apparatus and may be capable of demonstrating: formation of high resolution images; release from oil-less fusion rollers over a wide range of fusion temperature and print density; high transparency for OHP slides over a wide range of fusion temperature and print density; high transfer efficiency and the ability to clean any residual toner from the photoconductor, and the absence of filming of the metering blade, development roller and photoconductor over a long print run.

Throughout the description and claims of this specification, the words "comprise" and "contain" and variations of the words, for example "comprising" and "comprises", mean "including but not limited to", and are not intended to (and do not) exclude other components and/or steps.

Unless the context clearly indicates otherwise, plural forms of the terms herein are to be construed as including the singular form and vice versa.

It will be appreciated that variations to the foregoing embodiments of the invention can be made while still falling within the scope of the invention. Each feature disclosed in this specification, unless stated otherwise, may be replaced by alternative features serving the same, equivalent or similar purpose. Thus, unless stated otherwise, each feature disclosed is one example only of a generic series of equivalent or similar features.

All of the features disclosed in this specification may be combined in any combination, except combinations where at least some of such features and/or steps are mutually exclusive. In particular, the preferred features of the invention are applicable to all aspects of the invention and may be used in any combination. Likewise, features described in non-essential combinations may be used separately (not in combination).

It will be appreciated that many of the features described above, particularly of the preferred embodiments, are inventive in their own right and not just as part of an embodiment of the present invention. Independent protection may be sought for these features in addition to or alternative to any invention presently claimed.

The invention will now be illustrated by the following Examples, which are non-limiting on the scope of the invention. All percentages or parts referred to are percentages or parts by weight unless otherwise stated. The solids content quoted for the dispersions in these examples includes any surfactant present in the dispersion.

18

## EXAMPLE 1

## Preparation of Latexes

## EXAMPLE 1.1

## Synthesis of Low Molecular-Weight Latex (a-1)

10 A low molecular weight resin was synthesised by emulsion polymerisation. The monomers used were styrene (83.2 wt % of total monomers), 2-hydroxyethyl methacrylate (3.5 wt %) and acrylic ester monomers (13.3 wt %). Ammonium persulphate (0.5 wt % on monomers) was used as the initiator, and a mixture of thiol chain transfer agents (4.5 wt % on monomers) was used as chain transfer agents. The surfactant was Akypo<sup>TM</sup> RLM100 (a carboxylated alkyl ethoxylate, i.e. a carboxy-functional surfactant, available from Kao, 3.0 wt % 15 on monomers). The emulsion had a particle size of 77 nm, and a Tg midpoint (as measured by differential scanning calorimetry (dsc)) of 59° C. GPC analysis against polystyrene standards showed the resin to have Mn=6,300, Mw=14,400, Mw/Mn=2.29. The solids content of the latex dispersion (a-1) 20 was 30 wt %.

## EXAMPLE 1.2

## Synthesis of Low Molecular-Weight Latex (a-2)

30 A low molecular weight resin was synthesised by emulsion polymerisation. The monomers used were styrene (83.2 wt %), 2-hydroxyethyl methacrylate (3.5 wt %) and acrylic ester monomers (13.3 wt %). Ammonium persulphate (0.5 wt % on monomers) was used as the initiator, and a mixture of thiol chain transfer agents (4.5 wt % on monomers) was used as chain transfer agents. The surfactant was Akypo<sup>TM</sup> RLM100 (3.0 wt % on monomers). The emulsion had a particle size of 89 nm, and a Tg midpoint (as measured by differential scanning calorimetry (dsc)) of 57° C. GPC analysis against polystyrene standards showed the resin to have Mn=6,200, Mw=14,800, Mw/Mn=2.39. The solids content of the latex 35 dispersion (a-2) was 30.6 wt %.

## EXAMPLE 1.3

## Synthesis of Medium Molecular-Weight Latex (a-3)

50 A bimodal molecular weight distribution latex was made by a two-stage polymerisation process, in which the higher molecular weight portion was made in the absence of chain transfer agent, and in which the molecular weight of the lower molecular weight portion was reduced by use of 2.5 wt % of mixed thiol chain transfer agents. Ammonium persulphate (0.5 wt % on monomers) was used as the initiator, and the surfactant was Akypo<sup>TM</sup> RLM100 (3.0 wt % on monomers). The monomer composition of the low molecular weight portion was styrene (82.5%), 2-hydroxyethyl methacrylate (2.5%) and acrylic ester monomers (15.0%). The overall monomer composition was styrene (73.85 wt %), 2-hydroxyethyl methacrylate (6.25 wt %) and acrylic ester monomers (19.9 wt %). The emulsion had a particle size of 81 nm. GPC 55 analysis against polystyrene standards showed the resin to 60

19

have Mn=33,000, Mw=704,000, Mw/Mn=21.3. The solids content of the latex dispersion (a-3) was 39.9 wt %.

## EXAMPLE 1.4

## Synthesis of Medium Molecular-Weight Latex (a-4)

A bimodal molecular weight distribution latex was made by a two-stage polymerisation process, in which the higher molecular weight portion was made in the absence of chain transfer agent, and in which the molecular weight of the lower molecular weight portion was reduced by use of 2.5 wt % of mixed thiol chain transfer agents. Ammonium persulphate (0.5 wt % on monomers) was used as the initiator, and the surfactant was Akypo<sup>TM</sup> RLM100 (3.0 wt % on monomers). The monomer composition of the low molecular weight portion was styrene (82.5%), 2-hydroxyethyl methacrylate (2.5%) and acrylic ester monomers (15.0%). The overall monomer composition was styrene (73.85 wt %), 2-hydroxyethyl methacrylate (6.25 wt %) and acrylic ester monomers (19.9 wt %). The emulsion had a particle size of 82 nm. GPC analysis against polystyrene standards showed the resin to have Mn=20,000, Mw=679,000, Mw/Mn=34.0. The solids content of the latex dispersion (a-4) was 40 wt %.

## EXAMPLE 2

## Pigment Dispersions

## EXAMPLE 2.1

## Magenta Pigment Dispersion (b-1)

A dispersion of CI Pigment Red 122 was used. The pigment was milled in water using a bead mill, with Akypo<sup>TM</sup> RLM100 (ex Kao) and Solisperse<sup>TM</sup> 27000 (ex Noveon) as dispersants. The solids content of the dispersion was 28.6 wt %.

## EXAMPLE 2.2

## Cyan Pigment Dispersion (b-2)

A dispersion of CI Pigment Blue 15:3 was used. The pigment was milled in water using a bead mill, with Akypo<sup>TM</sup> RLM100 and Solisperse<sup>TM</sup> 27000 as dispersants. The solids content of the dispersion was 27.3 wt %.

## EXAMPLE 2.3

## Magenta Pigment Dispersion (b-3)

A dispersion of CI Pigment Red 122 was used. The pigment was milled in water using a bead mill, with Akypo<sup>TM</sup> RLM100 and Solisperse<sup>TM</sup> 27000 as dispersants. The total solids of the dispersion was 28.8 wt %.

## EXAMPLE 3

## Wax Dispersions

## EXAMPLE 3.1

## Wax Dispersion (c-1)

A wax mixture comprising 80 parts by weight Paraflint C80 and 20 parts carnauba wax was melt dispersed in water, with Akypo<sup>TM</sup> RLM100. The solids content of the dispersion was 25.4%.

20

## EXAMPLE 3.2

## Wax Dispersion (c-2)

5 A wax mixture comprising 80 parts by weight Paraflint C80 and 20 parts carnauba wax was melt dispersed in water, with Akypo<sup>TM</sup> RLM100 (Kao). The total solids was 25.25%.

## EXAMPLE 4

## Wet-Cake of Carboxy Functional Compound

## EXAMPLE 4.1

## Wet-Cake of Carboxy Functional Compound (d-1)

10 A wet-cake (d-1) of BONTRON E88<sup>TM</sup> in water (ex Orient) was used, which had a solids (BONTRON E88) content of 21.4%. BONTRON E88 is an aluminium complex of an alkyl salicylic acid compound (i.e. a carboxy functional compound of Formula (1) in complex form).

## EXAMPLE 4.2

## Wet-Cake (d-2)

15 A wet-cake (d-2) of BONTRON E88<sup>TM</sup> in water (ex Orient) was used, which had a solids (BONTRON E88) content of 16.45%.

## EXAMPLE 5

## Toner Preparation

## EXAMPLE 5.1

## Toner 1 (Comparative)

## Mixing Step:

20 Latex (a-1) (610.3 g), Latex (a-4) (70.4 g), the pigment dispersion (b-3) (36.5 g), wax dispersion (c-2) (118.8 g) and water (1415 g) were mixed and stirred.

## Association and Particle Growth:

25 The temperature of the mixture was raised to 37° C. Over the course of 290 seconds the mixed dispersions were circulated through a high shear mixer and back into the vessel during which 4% sulphuric acid (250 g) was added into the high shear mixer. The pH had reduced to 1.7. The mixture was heated for the next 155 minutes (to a maximum temperature of 58.1° C.). The mixture was then cooled to 50° C. A solution of sodium hydroxide 0.5M was added over 14 minutes to raise the pH to 7.

## Coalescence Step:

30 The temperature of the mixture was then raised to 120° C. and held at this temperature for a total of 60 minutes with stirring before being cooled to room temperature. Coulter Counter<sup>TM</sup> analysis showed the mean volume particle size was 7.2  $\mu$ m, the GSD<sub>v</sub> was 1.31 and the GSD<sub>n</sub> was 1.41. Microscopic analysis showed the toner particles to be of uniform size and slightly irregular in shape.

21

EXAMPLE 5.2

Toner 2 (Comparative)

## Mixing Step:

Latex (a-1) (783.9 g), Latex (a-3) (90.4 g), the pigment dispersion (b-1) (47.8 g), wax dispersion (c-1) (153.7 g), wet-cake (d-1) (15.5 g) and water (1128.9 g) were mixed and stirred. The total content of the carboxy functional compound (BONTRON E88) was 1% based on the total weight of the compound and the solids content of the latex, pigment and wax dispersions.

## Association and Particle Growth:

The temperature of the mixture was raised to 37° C. Over the course of 270 seconds the mixture was circulated through a high shear mixer and back into the vessel during which 4% sulphuric acid (280 g) was added into the high shear mixer. The pH was reduced to 1.85 by the addition of the acid. The mixture was heated for the next 175 minutes to a maximum temperature of 55.4° C. The mixture was then cooled to 50° C. A solution of sodium hydroxide (0.5M) was added over 13 minutes to raise the pH to 7.

## Coalescence Step:

The temperature of the mixture was then raised to 120° C. and the mixture was held at this temperature for a total of 60 minutes with stirring before being cooled to room temperature. Using a 100  $\mu$ m aperture, Coulter Counter™ analysis of the toner particles in the dispersion showed the mean volume particle size was 6.1  $\mu$ m, the GSD<sub>v</sub> was 1.25 and the GSD<sub>n</sub> was 1.39. Microscopic analysis showed the toner particles to be of uniform size and slightly irregular in shape.

EXAMPLE 5.3

Toner 3

## Mixing Step:

Latex (a-1) (937.9 g), Latex (a-3) (108.2 g), the pigment dispersion (b-1) (58.8 g), wax dispersion (c-1) (190 g), wet-cake (d-1) (62.2 g), and water (863.7 g) were mixed and stirred. The total content of the carboxy functional compound (BONTRON E88) was 3.3% based on the total weight of the compound and the solids content of the latex, pigment and wax dispersions.

## Association and Particle Growth:

The temperature of the mixture was raised to 37° C. Over the course of 300 seconds the mixed dispersions were circulated through a high shear mixer and back into the vessel during which 4% sulphuric acid (280 g) was added into the high shear mixer. The pH had reduced to 2.28. The temperature of the mixture was heated for the next 188 minutes (experiencing a maximum temperature of 57.6° C.). The mixture was then cooled to 50° C. A solution of sodium hydroxide (0.5M) was added over 17 minutes to raise the pH to 7.

## Coalescence Step:

The temperature of the mixture was then raised to 120° C. and held at this temperature for a total of 60 minutes with stirring before being cooled to room temperature. Using a 100  $\mu$ m aperture, Coulter Counter™ analysis of the toner particles in the dispersion showed the mean volume particle size was 6.3  $\mu$ m, the GSD<sub>v</sub> was 1.21 and the GSD<sub>n</sub> was 1.26. Microscopic analysis showed the toner particles to be of uniform size and slightly irregular in shape.

EXAMPLE 5.2

Toner 2 (Comparative)

22

EXAMPLE 5.4

Toner 4

## 5 Mixing Step:

Latex (a-1) (938 g), Latex (a-3) (108.2 g), the pigment dispersion (b-1) (58.8 g), wax dispersion (c-1) (189.1 g), wet-cake (d-1) (62.2 g), Akypo™ RLM 100 (20 g, 40% solids) and water (843.68 g) were mixed and stirred. The total content of the carboxy functional compound (BONTRON E88) was 3.2% based on the total weight of the compound, the solids content of the latex, pigment and wax dispersions and the added surfactant (Akypo™ RLM 100).

## 15 Association and Particle Growth:

The temperature of the mixture was raised to 37° C. Over the course of 270 seconds the mixture was circulated through a high shear mixer and back into the vessel during which 4% sulphuric acid (280 g) was added into the high shear mixer. The pH was reduced to 2.06 by the addition of the acid. The mixture was heated for the next 220 minutes to a maximum temperature of 56.4° C. The mixture was then cooled to 50° C. A solution of sodium hydroxide (0.5M) was added over 11 minutes to raise the pH to 7.

## 25 Coalescence Step:

The temperature of the mixture was then raised to 120° C. and held at this temperature for a total of 60 minutes with stirring before being cooled to room temperature. Using a 100  $\mu$ m aperture, Coulter Counter™ analysis of the toner particles in the dispersion produced showed the mean volume particle size was 6.3  $\mu$ m, the GSD<sub>v</sub> was 1.25 and the GSD<sub>n</sub> was 1.25. Microscopic analysis showed the toner particles to be of uniform size and slightly irregular in shape.

EXAMPLE 5.5

Toner 5

## 40 Mixing Step:

Latex (a-2) (1482.8 g), the pigment dispersion (b-2) (84.4 g), Akypo RLM 100 (40 g, 40% solids in water), wet-cake (d-2) (97.3 g) and water (1110.7 g) were mixed and stirred. The total content of the carboxy functional compound BONTRON E88 was 3.2% based on the total weight of the BONTRON E88, the solids content of the latex and pigment dispersions and the added Akypo™ surfactant.

## 50 Association and Particle Growth:

The temperature of the mixture was raised to 48.4° C. Over the course of 325 seconds the was circulated through a high shear mixer and back into the vessel during which 4% sulphuric acid (225 g) was added into the high shear mixer. The pH was reduced to 2.36 by the addition of the acid. The mixture was heated for the next 176 minutes to a maximum temperature of 59.7° C. A solution of sodium dodecylbenzenesulphonate (120.0 g of a 10% solution) was added followed by dilute sodium hydroxide solution to raise the pH to 7.

## 60 Coalescence Step:

The temperature was then raised to 120° C. and held at this temperature for a further 45 minutes before being cooled to room temperature. Coulter Counter™ analysis of the toner particles produced showed the mean volume particle size was 7.8  $\mu$ m, the GSD<sub>v</sub> was 1.19 and the GSD<sub>n</sub> was 1.23. Microscopic analysis showed the toner particles to be of uniform size and of smooth, “potato” shape.

23

## EXAMPLE 5.6

Toner 6

## Mixing Step:

Latex (a-2) (1575 g), the pigment dispersion (b-2) (91.0 g), Akypo RLM 100 (40 g, 40% solids in water), wet-cake (d-2) (103.3 g) and water (982 g) were mixed and stirred. The total content of the carboxy functional compound BONTRON E88 was 3.2% based on the total weight of the BONTRON E88, the solids content of the latex and pigment dispersions and the added Akypo<sup>TM</sup> surfactant.

## Association and Particle Growth:

The temperature of the mixture was raised to 43° C. Over the course of 300 seconds the mixture was circulated through a high shear mixer and back into the vessel during which 4% sulphuric acid (250 g) was added into the high shear mixer. The pH was reduced to 2.01 by the addition of the acid. The mixture was heated for the next 190 minutes to a maximum temperature of 60.5° C. A solution of sodium dodecylbenzenesulphonate (127.5 g of a 10% solution) was then added followed by dilute sodium hydroxide solution to raise the pH to 7.

## Coalescence Step:

The temperature was then raised to 125° C. and held at this temperature for a further 45 minutes with stirring before being cooled to room temperature. Coulter Counter<sup>TM</sup> analysis of the toner particles produced showed the mean volume particle size was 7.1 µm, the GSD<sub>v</sub> was 1.18 and the GSD<sub>n</sub> was 1.20. Microscopic analysis showed the toner particles to be of uniform size and of smooth, "potato" shape.

## EXAMPLE 5.7

Toner 7

## Mixing Step:

Latex (a-1) (976.6 g), Latex (a-4) (112.7 g), the pigment dispersion (b-3) (58.33 g), wax dispersion (c-2) (190.1 g), Akypo RLM 100 (20 g, 40% solids) and water (698.8 g) were mixed and stirred.

In a separate bottle 2-hydroxy-3-naphthoic acid (13.32 g) was dissolved in a 150.32 g of sodium hydroxide (0.5M). The resultant solution was then added to the latex, pigment and wax mixture. Thus, the total content of carboxy functional compound (2-hydroxy-3-naphthoic acid salt) was 3.1% based on the total weight of carboxy functional compound, the solids content of the latex, pigment and wax dispersions and the added surfactant (Akypo<sup>TM</sup> RLM 100).

## Association and Particle Growth:

The temperature of the mixture was raised to 37° C. Over the course of 290 seconds the mixed dispersions were circulated through a high shear mixer and back into the vessel during which 4% sulphuric acid (280 g) was added into the high shear mixer. The pH had reduced to 2.1. The mixture was heated for the next 175 minutes (to a maximum temperature of 58.1° C.). The mixture was then cooled to 50° C. A solution of sodium hydroxide 0.5M was added over 16 minutes to raise the pH to 7.

## Coalescence Step:

The temperature of the mixture was then raised to 120° C. and held at this temperature for a total of 60 minutes with stirring before being cooled to room temperature. Coulter

24

Counter<sup>TM</sup> analysis showed the mean volume particle size was 7.0 µm, the GSD<sub>v</sub> was 1.24 and the GSD<sub>n</sub> was 1.23. Microscopic analysis showed the toner particles to be of uniform size and slightly irregular in shape.

5

## EXAMPLE 5.8

Toner 8

## Mixing Step:

Latex (a-1) (976.4 g), Latex (a-4) (112.7 g), the pigment dispersion (b-2) (58.4 g), wax dispersion (c-2) (190.1 g), Akypo RLM 100 (20 g, 40% solids) and water (735.0 g) were mixed and stirred.

In a separate bottle 3,5-di-tertbutylsalicylic acid (13.32 g) was dissolved in a 113.54 g of sodium hydroxide (0.5M). The resultant solution was then added to the latex, pigment and wax mixture. Thus, the total content of carboxy functional compound (3,5-di-tertbutylsalicylic acid salt) was 3.1% based on the total weight of carboxy functional compound, the solids content of the latex, pigment and wax dispersions and the added surfactant (Akypo<sup>TM</sup> RLM 100).

## Association and Particle Growth:

The temperature of the mixture was raised to 37° C. Over the course of 290 seconds the mixed dispersions were circulated through a high shear mixer and back into the vessel during which 4% sulphuric acid (280 g) was added into the high shear mixer. The pH had reduced to 1.9. The mixture was heated for the next 175 minutes (to a maximum temperature of 58.0° C.). The mixture was then cooled to 50° C. A solution of sodium hydroxide 0.5M was added over 15 minutes to raise the pH to 7.

## Coalescence Step:

The temperature of the mixture was then raised to 120° C. and held at this temperature for a total of 60 minutes with stirring before being cooled to room temperature. Coulter Counter<sup>TM</sup> analysis showed the mean volume particle size was 5.9 µm, the GSD<sub>v</sub> was 1.24 and the GSD<sub>n</sub> was 1.23. Microscopic analysis showed the toner particles to be of uniform size and slightly irregular in shape.

35

## EXAMPLE 5.9

Toner 9

## Mixing Step:

Latex (a-1) (976.4 g), Latex (a-3) (112.7 g), the pigment dispersion (b-3) (58.4 g), wax dispersion (c-2) (190.1 g) and water (718.8 g) were mixed and stirred.

In a separate bottle 2-hydroxy-3-naphthoic acid (13.32 g) was dissolved in a 150.32 g of sodium hydroxide (0.5M). The resultant solution was then added to the latex, pigment and wax mixture. Thus, the total content of carboxy functional compound (2-hydroxy-3-naphthoic acid salt) was 3.2% based on the total weight of carboxy functional compound and the solids content of the latex, pigment and wax dispersions added.

## Association and Particle Growth:

The temperature of the mixture was raised to 37° C. Over the course of 300 seconds the mixed dispersions were circulated through a high shear mixer and back into the vessel during which 4% sulphuric acid (280 g) was added into the high shear mixer. The pH had reduced to 2.24. The mixture was heated for the next 175 minutes (experiencing a maxi-

60

55

60

25

mum temperature of 57.1° C.). The mixture was then cooled to 50° C. A solution of sodium hydroxide 0.5M was added over 12 minutes to raise the pH to 7.

Coalescence Step:

The temperature of the mixture was then raised to 120° C. and held at this temperature for a total of 60 minutes with

26

5 The particle sizes and particle size distributions of the toners are shown in Table 1. It can be seen that the particle size distribution, as characterised by the GSD<sub>n</sub> and GSD<sub>v</sub> value, especially GSD<sub>n</sub>, is significantly narrower for the Toners made according to the present invention compared to the comparative Toners 1 and 2.

TABLE 1

| Example               | % wt Carboxy Functional Compound (acid or salt form) | % wt Carboxy Functional Compound (complex form) | % wt Carboxy Functional Compound (total) | Mean Volume Particle size (μm) | GSD <sub>v</sub> | GSD <sub>n</sub> |
|-----------------------|------------------------------------------------------|-------------------------------------------------|------------------------------------------|--------------------------------|------------------|------------------|
| Toner 1 (Comparative) | 0                                                    | 0                                               | 0                                        | 7.2                            | 1.31             | 1.41             |
| Toner 2 (Comparative) | 0                                                    | 1.0                                             | 1.0                                      | 6.1                            | 1.25             | 1.39             |
| Toner 3               | 0                                                    | 3.3                                             | 3.3                                      | 6.3                            | 1.21             | 1.26             |
| Toner 4               | 0                                                    | 3.2                                             | 3.2                                      | 6.3                            | 1.25             | 1.25             |
| Toner 5               | 0                                                    | 3.2                                             | 3.2                                      | 7.8                            | 1.19             | 1.23             |
| Toner 6               | 0                                                    | 3.2                                             | 3.2                                      | 7.1                            | 1.18             | 1.20             |
| Toner 7               | 3.1                                                  | 0                                               | 3.1                                      | 7.0                            | 1.24             | 1.23             |
| Toner 8               | 3.1                                                  | 0                                               | 3.1                                      | 5.9                            | 1.24             | 1.23             |
| Toner 9               | 3.2                                                  | 0                                               | 3.2                                      | 8.1                            | 1.29             | 1.27             |
| Toner 10              | 3.2                                                  | 1.0                                             | 4.2                                      | 8.0                            | 1.22             | 1.29             |

stirring before being cooled to room temperature. Coulter Counter™ analysis showed the mean volume particle size was 8.1 μm, the GSD<sub>v</sub> was 1.29 and the GSD<sub>n</sub> was 1.27. Microscopic analysis showed the toner particles to be of uniform size and slightly irregular in shape.

EXAMPLE 5.10

Toner 10

Mixing Step:

Latex (a-1) (964.9 g), Latex (a-4) (111.4 g), the pigment dispersion (b-3) (58.33 g), wax dispersion (c-2) (190.1 g), wet-cake (d-1) (18.7 g) and water (680) were mixed and stirred.

In a separate bottle 2-naphthoic acid (13.32 g) was dissolved in a 164.29 g of sodium hydroxide (0.5M). The resultant solution was then added to the latex, pigment, wax and wet cake mixture. Thus, the total content of carboxy functional compound was 4.2% (comprising 1% Bontron™ E88 complex from the wet cake and 3.2% 2-naphthoic acid salt) based on the total weight of carboxy functional compound and the solids content of the latex, pigment and wax dispersions.

Association and Particle Growth:

The temperature of the mixture was raised to 37° C. Over 50 the course of 290 seconds the mixed dispersions were circulated through a high shear mixer and back into the vessel during which 4% sulphuric acid (280 g) was added into the high shear mixer. The pH had reduced to 2.26. The mixture was heated for the next 155 minutes (to a maximum temperature of 58° C.). The mixture was then cooled to 50° C. A solution of sodium hydroxide 0.5M was added over 13 minutes to raise the pH to 7.

Coalescence Step:

The temperature of the mixture was then raised to 120° C. and held at this temperature for a total of 60 minutes with stirring before being cooled to room temperature. Coulter Counter™ analysis showed the mean volume particle size was 8.0 μm, the GSD<sub>v</sub> was 1.22 and the GSD<sub>n</sub> was 1.29. 65 Microscopic analysis showed the toner particles to be of uniform size and slightly irregular in shape.

25 The invention claimed is:

1. A process for the manufacture of a toner which comprises the steps of:
- providing a latex dispersion containing primary resin particles and surfactant;
  - providing a colorant dispersion containing primary colorant particles and surfactant;
  - optionally providing a wax dispersion containing primary wax particles and surfactant;
  - providing at least one carboxy functional compound of Formula (1), which may be in acid, salt and/or complex form:



Formula (1)

40 45 wherein R is a carbocyclic or heterocyclic radical which may be optionally substituted and Z<sub>1</sub> is a bond or linker group and wherein the amount of carboxy functional compound of Formula (1) provided is greater than 3% by weight, the amount of carboxy functional compound being calculated according to the following equation:

$$\begin{aligned} \text{amount of carboxy} \\ \text{functional compound} = \\ (\%) \text{ weight} \end{aligned}$$

$$\frac{100 \times \text{weight of carboxy functional compound}}{(\text{weight of carboxy functional compound} + \text{weight of solids content of latex, colorant and optional wax dispersions} + \text{weight of any additional surfactant})}$$

- 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 86

27

- f) causing the particles in the mixture to associate by adjusting the pH.
2. A process as claimed in claim 1 wherein R is selected from the group consisting of optionally substituted phenyl and optionally substituted naphthyl.
3. A process as claimed in claim 1 or 2 wherein the carboxy functional compound, which may be in acid, salt and/or complex form, has a Formula (2):



Formula (2)

where  $Z_2$  is a bond or linker group and A is an ionisable group.

4. A process as claimed in claim 3 wherein A is OH.
5. A process as claimed in claim 1 wherein the carboxy functional compound which may be in acid, salt and/or complex form is selected from the group consisting of: salicylic acid; substituted salicylic acid; hydroxy naphthoic acid and substituted hydroxy naphthoic acid.
6. A process as claimed in claim 1 wherein there is provided a mixture of two or more carboxy functional compounds of Formula (1) in step (d).

28

7. A process as claimed in claim 1 wherein the amount of carboxy functional compound in salt form and/or complex form is at least 1% by weight.
8. A process as claimed in claim 1 wherein the amount of carboxy functional compound in salt form and/or complex form is at least 3% by weight.
9. A process as claimed in claim 8 wherein the amount of carboxy functional compound is not more than 5% by weight.
10. A process as claimed in claim 1 wherein each of the latex, colorant and optional wax dispersions comprises a surfactant which contains a group which can be converted from an ionic to a non-ionic form and vice versa by adjusting the pH.
11. A process as claimed in claim 1 wherein after the association in step (f) the process comprises a further step (h) which comprises raising the temperature above the  $T_g$  of the resin to bring about coalescence of the particles.
12. A process as claimed in claim 1 wherein the volume average particle size of the toner is in the range from 2 to 20  $\mu\text{m}$  and the  $\text{GSD}_n$  value is not greater than 1.30.
13. A process as claimed in claim 12 wherein the  $\text{GSD}_n$  value is not greater than 1.28.
14. A process as claimed in claim 13 wherein the  $\text{GSD}_n$  value is not greater than 1.25.
15. A process as claimed in claim 1 wherein the carboxy functional compound of Formula (1) is an optionally substituted salicylic acid or a salt, or a complex thereof.

\* \* \* \* \*